

# UNITED STATES PATENT OFFICE.

OSKAR ELBERLING, OF FRANKENTHAL, GERMANY, ASSIGNOR TO FRANKENTHALER KESSELSCHMIEDE, VELTHUYSEN & CO., OF SAME PLACE.

## MODE OF COVERING SURFACES OF METAL WITH LEAD.

SPECIFICATION forming part of Letters Patent No. 395,269, dated December 25, 1888.

Application filed October 4, 1888. Serial No. 287,233. (No specimens.) Patented in Germany August 8, 1886, No. 38,897.

*To all whom it may concern:*

Be it known that I, OSKAR ELBERLING, a subject of the Emperor of Germany, and a resident at Frankenthal, Germany, assignor to the firm of FRANKENTHALER KESSELSCHMIEDE, VELTHUYSEN & CO., of Frankenthal, have invented new and useful Improvements in Covering Metallic Surfaces with Lead, of which the following is a specification.

This invention relates to an improved process of covering metallic articles, especially those of iron, with lead.

The surface of the article to be covered with lead is carefully cleaned in order to remove any oxide, dirt, and the like, (preferably by using steel brushes,) roughened by means of a sand-jet blower or the like, washed over with soldering-liquid, and then immersed in a hot-lead bath. While the article is in the lead bath the surface to be covered with lead is treated with steel brushes, whereby an intimate connection between the lead and iron is insured. The layer of lead produced in this manner on the surface of the article is, however, too thin to offer any resistance to the acids. Moreover, it is not uniform in consequence of the brushing, and must be covered by a second operation with a layer of lead which shall be of the desired thickness. The layer applied to the article in this second operation is welded or secured in a homogeneous manner upon the article previously covered with lead. For this purpose the article in the case of plane surfaces—for example, sheets or plates of iron—is placed horizontally upon a suitable support, washed over with soldering-liquid, and heated to about 400° centigrade. Molten lead is then poured upon the article and spreads uniformly over the entire horizontal surface. A border of a definite height, which has been previously placed around the surface, prevents the lead from passing over the edges of the latter and determines the thickness of the lead. After this the whole is again heated to a temperature above the melting-point of the lead for a longer or shorter time, according to the thickness of the article to be covered with lead. It is again treated with steel brushes in order to obtain an intimate con-

nnection of the leaded sheet or plate with the layer of lead to be applied to it, and is then allowed to cool, care being taken that during the cooling of the iron sheet or plate the lead above the latter shall be kept as long as possible at a temperature above the melting-point by the addition of more liquid lead. 55

In the case of articles which have no plane surface—for example, pipes, vessels, or boilers, and the like—the aforesaid second operation is carried out by placing the pipe vertically, providing a core of suitable material in its interior or a mold or casing around the same, and after the surface has been treated with 60 soldering-liquid heating it to 400° centigrade, and filling up the space between the wall and the core or casing with lead; then heating it again to a temperature above the melting-point of the lead and carefully cooling it, 65 fresh liquid lead being added from time to time.

The surfaces of articles treated in this manner present quite a homogeneous cover that is free from blisters and firmly adheres 75 to the article.

Having thus described my invention and the manner of employing the same, what I claim as my invention, and wish to have secured to me by Letters Patent of the United 80 States of America, is—

The herein-described process of coating articles of metal with lead, the same consisting in cleaning the surface of the article, then roughing the same, washing it with soldering-liquid, placing it in a bath of melted lead and at the same time treating the surface with stiff brushes, removing it from the bath, and after cooling washing it with soldering-liquid, 85 heating it to about 400° centigrade, applying 90 to and confining on the surface a layer of melted lead of a certain thickness, then heating it to a temperature above the melting-point of lead, and finally cooling it, substantially as set forth. 95

In testimony whereof I have signed my name to this specification in the presence of two subscribing witnesses.

OSKAR ELBERLING.

Witnesses:

E. D. COWEN,

J. L. SCLANDERS.